# EUROPEAN PATENT SPECIFICATION

(11) **EP 0 758 272 B1**
(45) Date of publication and mention of the grant of the patent: **03.03.1999**
(21) Application number: 95917633.0
(22) Date of filing: 21.04.1995
(51) Int. Cl.: B05D 1/12, B05D 1/28, B05D 1/06

(54) **SURFACE DEFECT DETECTION POWDER COMPOSITION, METHODS OF USING SAME AND APPLICATOR THEREFOR**
PULVERZUSAMMENSETZUNG ZUR DETEKTION OBERFLÄCHENFEHLER, IHRE VERWENDUNG UND APPLIKATOR
COMPOSITION EN POUDRE SERVANT A DETECTER DES DEFAUTS DE SURFACE, PROCEDES D'UTILISATION ET APPLICATION

(30) Priority: 06.05.1994 GB 9409015
(43) Date of publication of application: 19.02.1997
(73) Proprietor: MINNESOTA MINING AND MANUFACTURING COMPANY, St. Paul, Minnesota 55133-3427 (US)
(72) Inventor: BASTOW, David R., Harlow Essex CM19 5AE (GB)
(74) Representative: Bowman, Paul Alan
(86) International application number: US9504978
(87) International publication number: WO9530493

(56) References cited:
- WO-A-95/08405
- DE-A- 3 712 733
- PATENT ABSTRACTS OF JAPAN vol. 013 no. 135 (P-851) ,5 April 1989 & JP,A,63 304153 (TOKUSHU) 12 December 1988,
- PATENT ABSTRACTS OF JAPAN vol. 010 no. 169 (P-468) ,14 June 1986 & JP,A,61 022238 (CHIYUUGOKU) 30 January 1986,
- DATABASE WPI Week 9441 Derwent Publications Ltd., London, GB; AN 94-331367 & SU,A,91 936 325 (CHEM. TECHN. RES. INST.) , 7 June 1993
- DATABASE WPI Week 8625 Derwent Publications Ltd., London, GB; AN 86-162315 & US,A,6 772 815 (US. SEC. OF AIR FORCE) , 18 March 1986

## Description

### Technical Field

This invention relates to a powder composition for use in the detection of defects on surfaces and to its method of use in surface finishing processes. The invention also relates to an applicator means for dispensing and applying such a powder composition.

### Background Art

Many surface finishing processes, particularly repair processes in the automotive refinish industry, involve the application of fillers to imperfections in the surface followed by progressive abrasion with coarser to finer abrasive materials until the desired smooth surface is achieved. A series of protective coatings is applied, e.g., primer, paint coats, lacquers and so forth, and each layer is normally rubbed down prior to application of the next coat in order to ensure a smooth surface.

In order to assist the operator in identifying areas requiring abrasion and highlighting defects during the repair process, it is known to apply a guide coat to the surface being treated. The guide coats generally comprises a dilute paint mixture which is sprayed over the surface to be treated to provide a light paint coating. As the surface is abraded the guide coat is removed from the higher portions of the surface leaving the visible guide coat on the lower areas. Thus, the surface irregularities are clearly visible to the operator, enabling him to abrade and fill the appropriate areas.

The use of a dilute paint mixture as a guide coat suffers from the disadvantages that it is necessary to mask surrounding areas of surface which are not to be treated and the use of large amounts of volatile solvent is undesirable.

DE-A-3712733 which content forms the basis for the preamble of claims 1 and 8, discloses a metallic work blank which comprises an intermediate layer applied to the cleaned and roughened surface of the work blank to recognise defective spots. The intermediate layer contains an epoxide resin and between 3 and 10% of iron oxide.

Patent Abstracts of Japan P-851 vol. 013, 5 April 1989 discloses a coloured magnetic powder for magnetic particle testing which is produced by forming a film of a binder on the surface of the magnetic powder by mechanochemical reaction and then forming a film of coloured material likewise by mechanochemical reaction thereon.

WO95/08405 discloses application of a guide coat on a surface as part of a smoothing operation, e.g. of a vehicle bodywork, by distributing finely divided particulate material e.g. a non-toxic, water-based black powder paint, over the surface so the material remains on the surface and thus highlights any irregularities on the surface.

The present invention, described hereinafter, provides an alternative system for use as a guide coat.

According to the present invention there is provided an adhesive-free, dry, free-flowing powder composition suitable for use in surface defect detection. The invention powder composition comprises a physical mixture of particles of a colorant and particles of an extender, which mixture includes particles of colorant and particles of extender each having a particle size of less than 100µm.

The powder compositions of the invention provide a simple, effective guide coat which readily highlights surface imperfections, such as scratches, orange peel effect and dry over-spray. The compositions do not require the presence of solvents and therefore there is no drying time and the surface may be abraded immediately after application of the guide coat. Furthermore, it has been found that many powder compositions of the invention can substantially reduce the abrading time compared to the use of a guide coat formed by a dilute paint mixture.
Figure 1 represents a perspective view of an applicator for a powder composition in accordance with the invention.
Figure 2 represents a cross-section through a reservoir of powder composition.

The powder compositions of the invention are free from adhesive, thereby readily allowing the composition to be distributed readily over a large surface area.

Generally, at least 50%, preferably at least 90% by weight of the particles of the powder composition have a nonzero particle size of less than 100µm, in order to reveal defects in a surface having dimensions up to 100µm. Preferably the average particle size of all the particles used is less than 40µm, more preferably substantially all the particles have a particle size less than 40µm. It is preferred that the compositions contain some particles less than 10µm in particle size order to reveal fine scratches. More preferably the average particle size of the powder composition, overall, is about 10µm. In the present invention, by the terminology "particle size", it is meant the greatest cross-sectional diameter of the particle. These particle sizes can be determined by sieve tray screening.

The colorant is selected to contrast with the surface to which the composition will be applied. In principle, any dry, free-flowing colored particles may be used in the compositions of the invention. However, many organic pigments or dyes are not economical and/or do not spread evenly over the surface. Inorganic colorants are preferred, e.g., carbon black, iron oxide, etc. The most preferred colorant is carbon black, particularly activated carbon black. Mixtures of colorant may be employed.

The extender is generally a light-colored particulate material which dilutes the colorant. Suitable extenders include calcium carbonate, titanium dioxide, talc, magnesium stearate, zinc stearate, calcium stearate and aluminium stearate. The preferred extender in terms of economy and performance is calcium carbonate. Mixtures of extenders may be employed.

The morphology of the particles is not believed to be important providing the particles are free-flowing and will spread evenly. The colorant is generally present in an amount of less than 50% by weight of the composition and is preferably in the range 25 to 40% by weight.

A preferred guide coat composition of this invention comprises about 30-40% by weight carbon black(s) (total, if a combination is used) and about 60-70% by weight calcium carbonate. One preferred guide coat composition of the present invention is formulated to involve a physical mixture, by weight, of about 66% calcium carbonate (e.g., Snowcal™ 30); about 6% of a first type of carbon black (e.g., Raven™ 2000D); and about 28% a second type of carbon black except that it is an activated carbon black (e.g., Chemviron Type C). Snowcal™ 30 calcium carbonate powder can be commercially obtained from Croxton & Garry Ltd., Dorking, Surrey England, and is composed of 96% calcium carbonate, 2.0% silica, 0.1% ferric oxide, 0.2% alumina, and small residue of copper and lead. As to its physical properties, Snowcal™ 30 has a weight medium diameter of 4.6 µm; a specific gravity of 2.7; oil absorption (rub out method) of 15g/100g; and the percentage (%) retained on 125 µm sieve is 0.2, % retained on 63 µm sieve is 5.0, and & retained on 45 µm sieve is 12, with the % by weight of particles finer than 2 µm being 30. Raven™ 2000D carbon black powder, commercially available from Columbia Chemicals Co., Atlanta GA., USA, has a particle size of 18 nm (i.e., the arithmetic mean particle size as measured by electron microscopy); a surface area of about 200 m²/g; a DBP oil absorption of 70 cc/100g; and a powder density of 16 lb./ft³ (i.e. 2.57 x 10⁻² g/cm³). Chemviron Type C activated carbon black is commercially available from Chemviron Carbon Limited, Southlink Great Britain, and is a powder activated carbon having iodine number of 900 minutes; a moisture content of 2% maximum; an ash content of 14% maximum; a bulk density of 0.3 to 0.7 g/cm³; and a wet screen analysis through 325 US mesh (approximately 44 µm opening size) of 65 to 85%.

Desirable guide coat compositions would include those achieving as many as possible of the following desired characteristics:
safe to use;
ready to use (no mixing/preparation);
clean to use (not messy);
quick to use (covers the area quickly);
easy to see on surfaces (must be able to see
before and during sanding);
can be used on all sandable surfaces;
easy to remove excess;
over-paintable;
does not damage;
heat resistant;
must not load/clog abrasive;
low cost;
must not deleteriously influence sanding time;
must spread evenly;
needs to look good once applied;
easy to remove during sanding; and
swarf must not stain the newly sanded surface.

In practice, mixtures of carbon black and chalk of this invention are highly suitable as they fulfill most of these desired properties and are economical as compared with other materials.

The powder composition may be distributed over the surface by any suitable means, e.g., by sprinkling powder onto the surface and spreading with a cloth, pad or sponge. Only small amounts of powder composition are required and it is possible to apply a guide coat to the complete body work of a medium-sized automobile using about 9 grams of powder composition. In practice, the powder composition is generally employed in amounts of from 0.5 to 10g/m² based on the amount of colorant and extender having a particle size of less than 100µm.

The powder composition will generally be applied to surfaces to which filler has been applied and/or coated with primer, paint lacquer, and so forth, since these are the stages in the refinish industry where guide coats are generally employed. However, the guide coat compositions may be applied directly to non-treated surfaces if required, e.g., wood, metal, such as steel, plastic, fibre glass, and the like.

The powder composition may be stored and dispensed onto the surface from a bag, sachet or container similar to a salt or pepper shaker. Alternatively, the powder composition may be impregnated within the fibres of a fleece, mop, woven or non-woven fabric, or foam which may be wiped over the surface to deposit the powder. In a further embodiment the powder composition may be contained within the reservoir of an applicator and dispensed when the applicator is wiped over the surface. In another embodiment the powder is stored in a reservoir adapted to accommodate the applicator in order to load the applicator with powder prior to use. It is also possible to apply the powder material in a gas stream.

The invention will now be described with reference to the accompanying drawings of Figures 1 and 2.

As illustrated in Figure 1, the applicator means (1) comprises a handle (2) secured to a back-up pad (4) which supports an applicator pad (6). The handle (2) and back-up pad (4) also can be an integral molded body, such as a single integral element of molded rigid foam. The applicator pad (6) may comprise a mop, fleece or foam. A preferred applicator pad is formed of Caligen™ 4200 polyester polyurethane foam. Preferably the applicator pads are removable from the back-up pad in order that they may be replaced. Any suitable fixing system may be employed such as those commonly used for attaching abrasive paper to the back-up pads of sanding devices. For example, the foam may be coated with a pressure-sensitive adhesive and adhered to the back-up pad. Alternatively the pad may be laminated to brushed nylon on one surface which cooperates with a hook system provided on the surface of the back-up pad. For instance, the applicator can comprise a a layer of molded foam onto which the brushed nylon is laminated to the backside thereof. This brushed nylon, as described above, provides an attachment surface for the hooks of the back-up pad.

In one embodiment of the invention the powder is applied to the applicator pad (6), then applied to a surface, or, the powder is applied directly to the surface to be coated from a separate container.

In a further embodiment of the invention the handle (2) may be hollowed to provide a space for storing a supply of dry guide coat powder. Such a powder storage handle can be associated with a delivery system which will feed powder through the back-up pad (4) and applicator pad to allow application of the powder to a surface. The delivery system may comprise one or more holes through the back-up pad, which may be selectively opened and closed. Alternatively, a feed mechanism such as an Archimedes' screw or a power-assisted mechanism using a spring or compressed gas or propellant may facilitate delivery of the powder from the reservoir to the applicator pad.

In a further embodiment of the invention the applicator pad may be impregnated or loaded with the powder composition and thereafter attached to the back-up pad prior to use.

In another embodiment the applicator pad may be loaded with powder prior to use by use of a refill container device as shown in Figure 2. The refill container (8) comprises two basic components: an applicator pad support and powder delivery element (10) and a removable hollow cap (15) for storage of powder (12). The element (10) can be an integral member of molded rigid plastic comprising an open end (14); a horizontal, circular apertured surface (20) (such as having radial slot openings or channels (11) therethrough) having a horizontal annular flange (16) at its periphery; an upstanding circumferential rim (18) on its front side; and an upstanding circumferential flange (17) on its back side to permit removable attachment of removable cap element (15) which serves as a storage reservoir for refill powder (12). The outside surfaces of such flange (17) are ribbed to allow for interlocking with protrusion (13) provided on the inside wall of cap member (15), to allow these two members to be removably held together and detachable. The rim (18) is dimensioned to accommodate the applicator pad (6) of the applicator therewithin such that the pad may be supported on the horizontal flange (16). Preferably, the rim (18) has a plurality of circumferentially-spaced lugs or inward projections (tabs) (19) provided on the upper end of the rim (18) to assist in retaining an applicator pad during powder refill or handling. These lugs can be spaced equidistantly around the circumference of the rim end surfaces. The horizontal apertured surface (20) extends across the opening to provide additional support for the applicator pad (6). The element (20), alternatively, can be provided as a separate component attached to the upper surfaces of flange 16, such as where the element (20) is mesh or gauze.

The refill device (8) provides a useful support and replacement powder storage device for the applicator which prevents contamination of the applicator pad (6). The applicator pad (6) is readily loaded with powder by simply inverting or shaking the refill device (10) and applicator assembly, as fitted together. The presence of a uniform array of apertures, such as a plurality of radial slots (11) (e.g., radially eminating from a center of surface (20)) or in mesh or gauze, in element (20), assists in uniform loading of the powder over the surface of the applicator pad (6).

In one mode of the refill device of the invention, a removable, non-apertured separator sheet (not shown) can be interposed between surface (20), and a replacement applicator pad itself (not shown) and similar to pad (6) that is prepackaged within and provided as part of the refill device (8) when sold in commerce, so as to prevent powder flow from the cap reservoir into the replacement pad before usage of the refill device.

The powder composition is readily spread over a surface by application of light pressure to wipe the applicator pad over a surface.

The invention will now be illustrated by the following Examples in which all percentages are by weight unless otherwise indicated.

### Test Method

Each powder composition was tested on a primed Rover™ 200 bonnet (hood of an automobile) within 24 hours of painting. All work was carried out on a bench with the bonnets in a horizontal plane.

### 1. Bonnet Preparation

The surfaces were sanded with 3M 255P P180 HOOKIT™ 150mm diameter, 6 hole discs, one per bonnet, using a D/A 5mm orbital sander with dust extraction.

The swarf was removed with a solvent wipe.

A two-component "2K" primer, described below, was then applied and cured. The primer used was beige in color and comprised:
3 parts Standox™ 2K HS Filler (Part No. 020 78325), and
1 part Standox™ 2K Hardener for 2K Filler (Part No. 020 82594);
   each commercially available from Herberts, Essex, United Kingdom.

### 2. Guide Coat Application

- Powder:: 1 gram was sprinkled onto the surface and wiped over by hand with a foam pad.
- Aerosol:: A light coating of paint was applied to the primed surface.

### 3. Coating Appearance

The bonnets coated with powder were then compared with that of an aerosol guide coated panel.

### 4. Sanding

The guide coated surfaces were sanded with 3M 255P P500 HOOKIT™ 150mm diameter, 6 hole discs, one per bonnet, using a D/A 5mm orbital sander with dust extraction until a visually uniform sanded surface was attained. The areas and the time taken to sand were measured and recorded.

### Example 1-(Comparative)

### Sanding Time For Aerosol Guide Coated Panels

An aerosol guide coated bonnet was used as a control. The aerosol paint used was Spectra™ Cellulose Matte Black Spray Paint (Part No. SIMP 17) commercially available from Simoniz International plc, Cornwall, United Kingdom. This product has heretofore been used regularly in United Kingdom body shops as a guide coat. The data from eight experiments on the bonnets were analyzed to establish an overall average sanding time and to give an indication of the deviation of that data from the average. The information can be summarized as follows:
- Average Sanding Time per Unit Area: 5.82 minutes/m²
- Sample Standard Deviation(s): 0.50

These results were used as a control for the following experiments.

### Example 2

### Carbon Black and Calcium Carbonate Powder Guide Coats

The following materials were tested as guide coats:
Carbon black designated product "R2500" commercially available from Columbian Chemicals.
Carbon black designated product "R410" commercially available from Columbian Chemicals.
Carbon black "Type CBX" activated carbon black, wet screen analysis through 325 US mesh (45µm) = 96%, commercially available from Chemviron Carbon Limited.
Carbon black "Type C" a powder activated carbon black, wet screen analysis through 325 US mesh (45µm) = 65 to 85%, commercially available from Chemviron Carbon Limited.
Calcium carbonate, Snowcal™ 20 commercially available from Croxton & Garry Limited, median diameter 4.6µm, percentage retained on 45µm sieve = 12% by wt.
Calcium carbonate, Snowcal™ 30 commercially available from Croxton & Garry Limited, median diameter 4.6 µm, percentage retained on 45µm sieve = 12% by wt.
Calcium carbonate, Snowcal™ 60 commercially available from Croxton & Garry Limited, median diameter 2.8µm, percentage retained on 45µm sieve = 0.02% by wt.

The following 31 different guide coat compositions summarized in Table 1 were prepared by mixing the indicated proportions (in wt.%) of each of carbon black and calcium carbonate. The guide coat compositions summarized in Table 1 were prepared, where, for each composition, the amount by weight % of carbon black contained is indicated in the left-hand column and the amount by weight % of calcium carbonate contained therewith is indicated in the adjacent right-hand column.

**Table 1**

| Carbon Black | Calcium Carbonate |
|---|---|
| 5% R2500 | 95% Snowcal™ 20 |
| 7% R2500 | 93% Snowcal™ 20 |
| 11% R2500 | 89% Snowcal™ 20 |
| 10% R2500 | 90% Snowcal™ 20 |
| 10% R2500 | 90% Snowcal™ 20 |
| 15% R2500 | 85% Snowcal™ 20 |
| 20% R2500 | 80% Snowcal™ 20 |
| 20% R2500 | 80% Snowcal™ 20 |
| 30% R2500 | 70% Snowcal™ 20 |
| 35% R2500 | 65% Snowcal™ 20 |
| | |
| 5% R410 | 95% Snowcal™ 20 |
| 10% R410 | 90% Snowcal™ 20 |
| 15% R410 | 85% Snowcal™ 20 |
| 20% R410 | 80% Snowcal™ 20 |
| 25% R410 | 75% Snowcal™ 20 |
| 27% R410 | 73% Snowcal™ 20 |
| 35% R410 | 65% Snowcal™ 20 |
| | |
| 25% Type CBX | 75% Snowcal™ 20 |
| 30% Type CBX | 70% Snowcal™ 20 |
| 30% Type CBX | 70% Snowcal™ 20 |
| 30% Type CBX | 70% Snowcal™ 30 |
| 30% Type CBX | 70% Snowcal™ 60 |
| 32.5% Type CBX | 67.5% Snowcal™ 20 |
| 35% Type CBX | 65% Snowcal™ 20 |
| 35% Type CBX | 65% Snowcal™ 20 |
| 37.5% Type CBX | 62.5% Snowcal™ 20 |
| 42.5% Type CBX | 57.5% Snowcal™ 20 |
| 45% Type CBX | 55% Snowcal™ 20 |
| | |
| 30% Type C | 70% Snowcal™ 20 |
| 30% Type C | 70% Snowcal™ 30 |
| 30% Type C | 70% Snowcal™ 60 |

The guide coat compositions described above in Table 1 were evaluated by the test method described above. All of the above compositions proved to be acceptable as guide coats having a sanding time per unit area in the range 3.5 to 5 minutes, which is less than the average time required using conventional aerosol paint as a guide coat.

Compositions having higher carbon black content were darker but provided no obvious advantage in terms of sanding time. Activated carbon black was more effective than non-activated carbon black. Composition comprising 25 to 40% by weight carbon black are preferred in terms of acceptable performance and economy.

The sanding performance of five dry powder guide coat systems was compared with a black aerosol guide coat using the above test method. The powders for each test powder sample of this example comprised 30% by weight carbon black and 70% by weight calcium carbonate. The results are indicated in Table 2.

**Table 2**

| Black Guide Coats | Sanding Time Per Unit Area (minutes/m²) |
|---|---|
| Type CBX/Snowcal™ 20 | 4.34 |
| Type CBX/Snowcal™ 60 | 4.36 |
| Type C/Snowcal™ 20 | 4.45 |
| Type C/Snowcal™ 30 | 3.63 |
| Type C/Snowcal™ 60 | 3.56 |
| Simoniz, Aerosol (control) | 5.82 |

### Example 3 (Comparative)

### Powder Paint Evaluations

This experiment investigated whether powder paints, in the form of the water dispersible products currently available in many retail stores, would be suitable as guide coats. The black powder paints used generally comprise a mix of pigment (carbon black), adhesive (starch) and filler (calcium carbonate); their proportions vary depending upon their end use and the manufacturer. Black powder paints from the Early Learning Centre (ELC), Calder Colours and Partners were used. The test method described above was again used. The results are summarized in Table 3.

**Table 3**

| Black Guide Coats | Sanding Time Per Unit Area (minutes/m²) | Application Comments | Sanding Comments |
|---|---|---|---|
| ELC, Powder | 6.06 | too dark, streaky coating | swarf stains, marks left on paint |
| Calder, Playgroup Powder | 6.16 | too dark, streaky coating | swarf stains, marks left on paint |
| Calder, Art Powder | 5.79 | too dark, streaky coating | swarf stains, marks left on paint |
| Partners, Powder | 6.29 | too dark, streaky coating | swarf stains, marks left on paint |

The appearance of the bonnets coated with the powder paints were unacceptable when compared with the aerosol spray paint guide coated bonnet. The coatings were too dark and very streaky.

The swarf created while sanding the bonnets coated with the powder paints stained the newly sanded surfaces. All the bonnets coated with the powder paints took longer to sand than the aerosol spray paint guide coated bonnet.

### Example 4

### Comparison of Different Powders

The following powders were tested as guide coats:
Carbon Black Type C;
Snowcal™ 20;
Talc;
30% Carbon Black Type MT, 70% Snowcal™ 20;
30% Carbon Black Type C, 70% Talc;
30% Carbon Black Type C, 70% Magnesium Stearate;
30% Carbon Black Type C, 70% Stearic Acid;
30& Carbon Black Type C, 70% Titanium Dioxide;
30% Carbon Black Type C, 70% Zinc Stearate 30%;
Carbon Black Type C, 70% Calcium Stearate 30%; and
Carbon Black Type C, 70% Aluminium Stearate.

In Table 4, the results observed upon subjecting each of the above powder formulations to the test method are summarized. The mixing proportions, if any, as described above for the various powder formulations studied for this example, are omitted from Table 4 merely for the sake of brevity.

**Table 4**

| Guide Coats | Sanding Time per Unit Area (minutes/m²) | Comments |
|---|---|---|
| Type C | 4.80 | too dark, streaky |
| Snowcal™ 20 | ∼3.8 | too light, difficult to evaluate |
| Talc | ∼3.62 | too light, difficult to evaluate |
| Type MT/Snowcal™ 20 | 3.76 | |
| Type C/Talc | 3.80 | difficult to evaluate |
| Type C/Stearic Acid | 5.9 | forms spheres on surface |
| Type C/TiO₂ | 4.0 | |
| Type C/Zn Stearate | 4.5 | |
| Type C/Ca Stearate | 4.2 | |
| Type C/A1 Stearate | 5.9 | |

All the powder guide coated panels sanded faster than the aerosol spray paint guide coated panel.

It was difficult to decide whether the bonnet coated with Snowcal™ 20 and the bonnet coated with talc were completely sanded as their coatings were almost invisible. Defects were undetectable on the bonnets coated with Snowcal™ 20 and talc, the powders were unable to highlight them.

Whilst talc, TiO₂ and stearates may be used as extenders they do not appear to offer advantages over calcium carbonate.

### Example 5

### Colored Guide Coats

Tests were conducted using compositions consisting of 30% colorant and 70% Snowcal™ 30 (by wt.), with the colorant changed as indicated in the following descriptions of the compositions studied:

The colorants each used with 70% Snowcal™ 30 were:
Sico Red L3750, an organic colorant commercially available from BASF.
Milori Blue L6697, an inorganic colorant commercially available from BASF.
Heliogen Blue L6920 a phthalocyanine commercially available from BASF.
Calder Colours Green Art Powder Paint and iron oxide red, Bayferrox 120 commercially available from BASF. The powders were subjected to the above test method and the results are summarized in Table 5.

**Table 5**

| Guide Coat | Sanding Time per Unit Area (minutes/m²) | Comments |
|---|---|---|
| Sico Red/Snowcal™ 30 | 6.8 | too dark |
| Heliogen Blue/Snowcal™ 30 | 7.0 | too dark, swarf stains |
| Green Art Powder/Snowcal™ 30 | ∼3.8 | too light, difficult to evaluate |
| Red Iron oxide/Snowcal™ 30 | 4.8 | dark |
| Milori Blue/Snowcal™ 30 | 5.9 | too dark, swarf stains |
| Simoniz, Aerosol. (control) | 5.82 | |

Whilst all the guide compositions were useful to some degree, the colorants tested did not appear to be optimal as compared to carbon black. Iron oxide was the best alternative to carbon black.

## Claims

1. A composition suitable for use in surface defect detection characterised in that the composition is an adhesive-free, dry, free-flowing powder comprising particles of a colourant and particles of an extender, wherein said particles of colourant and said particles of extender each include fine particles having a particle size of less than 100µm.

2. A composition as claimed in Claim 1 characterised in that the average particle size of all said particles is less than 40µm.

3. A composition as claimed in Claim 1 or Claim 2 characterised in that it comprises fine particles having a particle size less than 10µm.

4. A composition as claimed in any preceding Claim characterised in that said colourant is selected from the group consisting of carbon black and iron oxide and said extender is selected from the group consisting of calcium carbonate, titanium dioxide, talc, magnesium stearate, zinc stearate, calcium stearate and aluminium stearate.

5. A composition as claimed in Claim 1 characterised in that the colourant comprises activated carbon black and said extender comprises calcium carbonate.

6. A composition as claimed in any preceding Claim characterised in that it consists essentially of from about 25% to about 40% by weight colourant and from about 60% to about 75% by weight of extender.

7. A composition as claimed in Claim 6 characterised in that it consists essentially of about 28% activated carbon black, about 6% non-activated carbon black, and about 66% by weight of calcium carbonate.

8. A method of forming a guide coat on a surface to detect defects thereon characterised in that the method comprises distributing over the surface a powder composition as defined in any one of Claims 1 to 7.

9. A method as claimed in Claim 8 characterised in that it comprises the additional step of sanding the guide coated surface.

10. A surface bearing a guide coat characterised in that the guide coat comprises a powder composition as defined in any one of Claims 1 to 7.

11. A surface bearing a guide coat as claimed in Claim 10 characterised in that said surface is part of an automobile body.

12. Apparatus (1) for applying a guide coat to a surface to detect defects thereon comprising an applicator pad (6) effective to support and apply a powder composition as defined in any one of Claims 1 to 7.

13. Apparatus as claimed in Claim 12 characterised in that the applicator pad (6) is impregnated with said dry powder composition.

14. Apparatus as claimed in Claims 12 or 13 characterised in that it further comprises a handle (2) secured to a back-up pad (4) which supports said applicator pad (6), and further characterised by a reservoir located inside said handle (2) containing the dry powder composition and a delivery means capable of feeding said powder composition through said back-up paid (4) to deliver powder from the reservoir to said applicator paid (6).

15. A powder applicator refill device comprising:
an applicator pad and powder delivery element (10) and powder storage cap (15) removably attached to said element (10), wherein said element (10) is comprised of (i) a horizontal, circular aperture surface (20) having a front side and a back side with a horizontal annular flange at its periphery, (ii) an upstanding circumferential rim (18) extending from the periphery of the front side of said surface (20) having a plurality of lugs formed at upper ends of said rim (18) which project inward; (iii) an upstanding circumferential flange (17) extending from the back side of said surface (20) adapted to removably interfit and interlock with said cap (15).

16. The refill device as claimed in Claim 15 characterised in that it further comprises a powder composition as defined in any one of Claims 1 to 7 contained within cap (15), and a powder applicator pad (6) positioned within element (10) and on flange (16).

## Patentansprüche

1. Zusammensetzung, geeignet zur Verwendung für die Feststellung von Oberflächenfehlern, dadurch gekennzeichnet, daß die Zusammensetzung ein klebstofffreies, trockenes, freifließendes Pulver ist, umfassend Teilchen aus einem farbgebenden Mittel und Streckmittel-Teilchen, wobei die Teilchen aus einem farbgebenden Mittel und die Streckmittel-Teilchen jeweils feine Teilchen mit einer Teilchengröße von weniger als 100 µm umfassen.

2. Zusammensetzung nach Anspruch 1, dadurch gekennzeichnet, daß die mittlere Teilchengröße aller Teilchen weniger als 40 µm beträgt.

3. Zusammensetzung nach Anspruch 1 oder Anspruch 2, dadurch gekennzeichnet, daß sie feine Teilchen mit einer Teilchengröße von weniger als 10 µm umfaßt.

4. Zusammensetzung nach einem der vorhergehenden Ansprüche, dadurch gekennzeichnet, daß das farbgebende Mittel aus der aus Ruß und Eisenoxid bestehenden Gruppe ausgewählt ist und das Streckmittel aus der aus Calciumcarbonat, Titandioxid, Talk, Magnesiumstearat, Zinkstearat, Calciumstearat und Aluminiumstearat bestehenden Gruppe ausgewählt ist.

5. Zusammensetzung nach Anspruch 1, dadurch gekennzeichnet, daß das farbgebende Mittel aktivierten Ruß umfaßt und das Streckmittel Calciumcarbonat umfaßt.

6. Zusammensetzung nach einem der vorhergehenden Ansprüche, dadurch gekennzeichnet, daß sie im wesentlichen aus etwa 25 Gew.-% bis etwa 40 Gew.-% farbgebendem Mittel und etwa 60 Gew.-% bis etwa 75 Gew.-% Streckmittel besteht.

7. Zusammensetzung nach Anspruch 6, dadurch gekennzeichnet, daß sie im wesentlichen aus etwa 28 Gew.-% aktiviertem Ruß, etwa 6 Gew.-% nicht aktiviertem Ruß und etwa 66 Gew.-% Calciumcarbonat besteht.

8. Verfahren zur Bildung einer Führungsschicht auf einer Oberfläche zum Nachweis von Fehlern darauf, dadurch gekennzeichnet, daß das Verfahren das Verteilen einer in einem der Ansprüche 1 bis 7 definierten Pulverzusammensetzung auf der Oberfläche umfaßt.

9. Verfahren nach Anspruch 8, dadurch gekennzeichnet, daß es den zusätzlichen Schritt des Schleifens der mit der Führung beschichteten Oberfläche umfaßt.

10. Oberfläche, die eine Führungsbeschichtung trägt, dadurch gekennzeichnet, daß die Führungsbeschichtung eine in einem der Ansprüche 1 bis 7 definierte Pulverzusammensetzung umfaßt.

11. Oberfläche, die eine Führungsbeschichtung trägt, dadurch gekennzeichnet, daß die Oberfläche Teil einer Kraftfahrzeug-Karosserie ist.

12. Vorrichtung (1) zum Auftragen einer Führungsbeschichtung auf eine Oberfläche zur Feststellung von Fehlern darauf, umfassend ein Auftragungskissen (6), das zum Halten und Auftragen einer in einem der Ansprüche 1 bis 7 definierten Pulverzusammensetzung wirksam ist.

13. Vorrichtung nach Anspruch 12, dadurch gekennzeichnet, daß das Auftragungskissen (6) mit der trockenen Pulverzusammensetzung imprägniert ist.

14. Vorrichtung nach Anspruch 12 oder 13, dadurch gekennzeichnet, daß sie weiterhin einen Handgriff (2) umfaßt, der an einem das Auftragungskissen (6) abstützenden Abstützelement (4) befestigt ist und weiterhin durch einen sich innerhalb des Handgriffs (2) befindlichen Vorratsbehälter gekennzeichnet ist, der die trockene Pulverzusammensetzung und ein Fördermittel umfaßt, mit dem die Pulverzusammensetzung durch die Abstützung (4) geführt werden kann, wodurch Pulver aus dem Vorratsbehälter zu dem Auftragungskissen (6) gefördert werden kann.

15. Pulverapplikator-Nachfüllvorrichtung, umfassend:
ein Auftragungskissen und ein Pulverförderelement (10) und einen Verschluß (15) zur Aufbewahrung des Pulvers, der lösbar an dem Element (10) befestigt ist, wobei das Element (10) aus (i) einer waagerechten, kreisförmigen, eine Öffnung aufweisenden Oberfläche (20) mit einer Vorderseite und einer Rückseite mit einem horizontalen, ringförmigen Flansch an ihrem Rand, (ii) einem aufragenden, sich vom Umfang der Vorderseite der Oberfläche (20) erstreckenden Umfangsrand (18) mit einer Mehrzahl von an den oberen Enden des Rands (18) ausgebildeten, nach innen ragenden Ansätzen; (iii) einem aufragenden, sich von der Rückseite der Oberfläche (20) erstreckenden Umfangsflansch (17), der so angepaßt ist, daß er mit dem Verschluß (15) lösbar zusammengreift und zusammenwirkt, besteht.

16. Nachfüllvorrichtung nach Anspruch 15, dadurch gekennzeichnet, daß sie weiterhin eine in einem der Ansprüche 1 bis 7 definierte, in dem Verschluß (15) enthaltene Pulverzusammensetzung und ein in dem Element (10) und auf dem Flansch (16) positioniertes Pulverauftragungselement (6) umfaßt.

## Revendications

1. Composition appropriée pour une utilisation dans la détection de défauts de surface, caractérisée en ce que la composition est une poudre fluide, sèche, exempte d'adhésif, comprenant des particules d'un colorant et des particules d'un diluant, dans laquelle lesdites particules de colorant et lesdites particules de diluant incluent chacune de fines particules ayant une granulométrie inférieure à 100 µm.

2. Composition selon la revendication 1, caractérisée en ce que la granulométrie moyenne de toutes lesdites particules est inférieure à 40 µm.

3. Composition selon la revendication 1 ou 2, caractérisée en ce qu'elle comprend de fines particules ayant une granulométrie inférieure à 10 µm.

4. Composition selon l'une quelconque des revendications précédentes, caractérisée en ce que ledit colorant est choisi dans le groupe formé par le noir de carbone et un oxyde de fer et ledit diluant est choisi dans le groupe formé par le carbonate de calcium, le dioxyde de titane, le talc, le stéarate de magnésium, le stéarate de zinc, le stéarate de calcium et le stéarate d'aluminium.

5. Composition selon la revendication 1, caractérisée en ce que le colorant comprend le noir de carbone actif et ledit diluant comprend le carbonate de calcium.

6. Composition selon l'une quelconque des revendications précédentes, caractérisée en ce qu'elle se compose essentiellement d'environ 25% à environ 40% en poids de colorant et d'environ 60% à environ 75% en poids de diluant.

7. Composition selon la revendication 6, caractérisée en ce qu'elle se compose essentiellement d'environ 28% de noir de carbone actif, d'environ 6% de noir de carbone non actif et d'environ 66% en poids de carbonate de calcium.

8. Procédé de formation d'un revêtement de guidage sur une surface pour y détecter les défauts, caractérisé en ce que le procédé comprend la distribution sur la surface d'une composition en poudre telle que définie selon l'une quelconque des revendications 1 à 7.

9. Procédé selon la revendication 8, caractérisé en ce qu'il comprend l'étape supplémentaire consistant à poncer la surface revêtue de guidage.

10. Surface supportant un revêtement de guidage, caractérisée en ce que le revêtement de guidage comprend une composition en poudre telle que définie selon l'une quelconque des revendications 1 à 7.

11. Surface supportant un revêtement de guidage selon la revendication 10, caractérisée en ce que ladite surface est une partie d'une carrosserie automobile.

12. Appareil (1) pour appliquer un revêtement de guidage à une surface pour y détecter les défauts comprenant un tampon applicateur (6) efficace pour supporter et appliquer une composition en poudre telle que définie selon l'une quelconque des revendications 1 à 7.

13. Appareil selon la revendication 12, caractérisé en ce que le tampon applicateur (6) est imprégné de ladite composition en poudre sèche.

14. Appareil selon la revendication 12 ou 13, caractérisé en ce qu'il comprend de plus une poignée (2) fixée à un patin support (4) qui supporte ledit tampon applicateur (6), et caractérisé de plus par un réservoir situé à l'intérieur de ladite poignée (2) contenant la composition en poudre sèche et un moyen de distribution capable d'alimenter ladite composition en poudre à travers le pain support (4) pour distribuer la poudre du réservoir audit tampon applicateur (6).

15. Dispositif de recharge d'applicateur de poudre comprenant:
un tampon applicateur et un élément de distribution de poudre (10) et une capsule de stockage de poudre (15) fixée de façon amovible dudit élément (10), dans lequel ledit élément (10) est composé (i) d'une surface d'ouverture circulaire, horizontale (20) ayant un côté frontal et un côté arrière avec une collerette annulaire frontale à sa périphérie, (ii) un rebord circonférentiel droit (18) s'étendant de la périphérie du côté frontal de ladite surface (20) ayant une pluralité d'oreilles formées aux extrémités supérieures dudit rebord (18) qui se projettent vers l'intérieur; (iii) une collerette circonférentielle droite (17) s'étendant du côté arrière de ladite surface (20) adapté pour s'ajuster entre eux de façon amovible et s'enclencher avec ladite capsule (15).

16. Dispositif de recharge selon la revendication 15, caractérisé en ce qu'il comprend de plus une composition de poudre telle que définie selon l'une quelconque des revendications 1 à 7, contenue dans la capsule (15), et un tampon applicateur de poudre (6) positionné dans l'élément (10) et sur la collerette (16).
